

## 1

3,036,969

## OIL CONTAINING RUST INHIBITING COMBINATION OF TWO INGREDIENTS

Ernest V. Wilson, Cranford, Henry R. Ertelt, Fanwood, and Willard H. Keeber, Westfield, N.J., assignors to Esso Research and Engineering Company, a corporation of Delaware

No Drawing. Filed Nov. 26, 1957, Ser. No. 698,937  
6 Claims. (Cl. 252—32.7)

The present invention is concerned with an oil containing two ingredients that in combination have surprising rust inhibiting properties. More specifically, this invention proposes the synergistic combination in an oil of minor amounts, under 0.2 weight percent each, of a branched alkyl mercaptoacetic acid and a non-emulsifying alkaline earth metal dialkylnaphthalene sulfonate to impart superior rust inhibition to the oil.

In brief compass, this invention proposes a lubricating composition comprising a major proportion of an oil of lubricating grade, and in the range of .005 to 1.0, e.g. 0.007 to 0.50, weight percent each of a C<sub>9</sub> to C<sub>17</sub> alkyl mercaptoacetic acid and an alkaline earth metal salt of a dialkylnaphthalene sulfonate, wherein each alkyl group has from 6 to 12 carbon atoms. The alkaline earth metal is preferably selected from the group of calcium and barium with the latter being most preferred. This rust inhibiting combination is particularly effective when used in proportions of 3.0 to 0.3 parts by weight of branched alkyl mercaptoacetic acid to 1 part by weight of alkaline earth dialkylnaphthalene sulfonate.

The mercaptoacetic acid used in the present composition has a formula:



wherein R is a branched alkyl group containing in the range of 9 to 17 carbon atoms. In a preferred embodiment of this invention R is highly branched. By "highly branched" is meant that the alkyl radical contains at least three forked or lateral groupings of one or more carbon atoms as side chains.

The particular naphthalene sulfonates used in this invention are characterized by the fact that in the concentrations used they do not tend to stabilize emulsions and in some cases actually act as demulsifying agents. That is, they do not promote the formation of stable emulsions as measured by the standard demulsibility test (ASTM D1401). Oils containing these naphthalene sulfonates do meet the limiting requirement for Navy turbine oils of 3 ml. maximum lacy cuff in 30 minutes as set forth in Specification MIL-L-17331A (Ships). The two alkyl groups of the alkyl naphthalene sulfonate may be located in various positions on the rings, and are branched chain radicals having from C<sub>6</sub> to C<sub>12</sub> carbon atoms per radical. Particularly preferred are the dinonylnaphthalene sulfonates of the type described in U.S. Patent 2,764,548.

The lubricating oil can be any conventional oil of lubricating grade known to the art, including animal, vegetable, synthetic and mineral oils—the latter being preferred. Preferably the oil base has a viscosity in the range of 37 to 150 seconds, Saybolt Universal at 210° F., a flash point above 370° F., a pour point below 25° F., and a gravity in the range of 26 to 34° API.

Examples of suitable synthetic oils are diesters such as di-2-ethyl hexyl sebacate; complex esters such as reaction products of 2 parts di-2-ethyl hexanol, 2 parts dibasic acid, and one part polyethylene glycol of about 200 average molecular weight; silicone oils such as the poly-

## 2

dimethyl siloxane Dow-Corning Fluid 200, prepared by hydrolytic condensation of dimethyl dichlorosilane; phosphorus derivatives such as C<sub>8</sub> Oxo diphenyl phosphate and the like.

5 The composition of this invention can also contain normal lubricating oil additives in their customary proportions to impart certain desired properties. These additives are known to the art and include viscosity index improvers, pour point depressants, extreme pressure agents, antioxidants, antifoamants and the like.

## EXAMPLE I

The base oil was derived from a Mid-Continent crude by phenol extraction, dewaxing by the MEK process with 15 methyl ethyl ketone and clay contacting.

It has the following inspections:

|                                               |        |
|-----------------------------------------------|--------|
| Viscosity, S.U.S., at 210° F. -----           | 59.5   |
| Viscosity, S.U.S., at 100° F. -----           | 393.5  |
| Viscosity index -----                         | 107    |
| 20 Flash point, ° F. -----                    | 485    |
| Pour point, ° F. -----                        | 20     |
| Color, Tag Robinson -----                     | 13½    |
| Conradson carbon -----                        | 0.02   |
| 25 Neutralization number as mg. KOH/gm. ----- | <0.01  |
| Saponification number -----                   | 0.07   |
| Sulfated ash, weight percent -----            | <0.001 |
| Sulfur, weight percent -----                  | 0.22   |

The additives were C<sub>13</sub> Oxo mercaptoacetic acid and 30 barium dinonylnaphthalene sulfonate. The alkyl radicals of the mercaptoacetic acid were derived from C<sub>13</sub> Oxo alcohol produced by carbonylation of tetrapropylene in the presence of a carbonyl catalyst, usually cobalt carbonyl, with carbon monoxide and hydrogen at a temperature

35 of from 200° to 400° C. and at a pressure of from 100 to 300 atmospheres. After the carbonylation stage, an aldehyde having one more carbon atom than the starting olefin is obtained, and this aldehyde is then hydrogenated at temperatures of from 150°—750° F. and at pressures of from 100—300 atmospheres, in the presence of a hydrogenating catalyst (copper, nickel, etc.) to obtain the C<sub>13</sub> Oxo alcohol. The C<sub>13</sub> Oxo alcohol may be converted to C<sub>13</sub> Oxo mercaptoacetic acid by reacting with hydrogen bromide to form the bromide and treating the bromide with an alkali metal mercaptan. The C<sub>13</sub> Oxo mercaptan is then reacted with sodium hydroxide. Monochloro acetic acid is added to this reaction mixture to produce the C<sub>13</sub> Oxo mercaptoacetic acid.

The barium dinonylnaphthalene sulfonate is prepared 50 by alkylating naphthalene with highly branched nonenes, for example, tripropylene with a suitable catalyst, such as, hydrogen fluoride or anhydrous aluminum chloride in an anhydrous solvent containing in solution the naphthalene. Suitable solvents such as naphtha, sulfur dioxide, nitrobenzene or a mixture of benzene and nitrobenzene in the alkylation result in a high yield of dinonylnaphthalene and relative ease of recovery of the solvent. The dinonylnaphthalene is then dissolved in an organic solvent which is substantially inert in its reaction with sulfuric acid and the solution is sulfonated with oleum or sulfuric acid. Barium carbonate is reacted with the dinonylnaphthalene sulfonic acid to form the barium dinonylnaphthalene sulfonate used in this invention.

Oil solutions were made up and tested in the MIL-L-65 17331A rust test. This test is the Standard ASTM sea water rust test (ASTM D665) and was carried out after distilled water washing of the oil sample at 90° C. for 30 minutes (as required by MIL-L-17331A (Ships)).

The results are shown in Table I.

3  
Table I

| Highly Branched C <sub>13</sub> Mercaptoacetic Acid (Weight percent) | Ba salt of (C <sub>6</sub> ) <sub>2</sub> Naphthalene Sulfonate (Weight percent) | MIL-L-17331A Rust Test |
|----------------------------------------------------------------------|----------------------------------------------------------------------------------|------------------------|
| 0.04                                                                 | Nil                                                                              | Fail (60% Rust).       |
| Nil                                                                  | 0.025                                                                            | Fail (20% Rust).       |
| Nil                                                                  | 0.05                                                                             | Fail (20% Rust).       |
| 0.015                                                                | 0.0075                                                                           | Pass (No Rust).        |
| 0.0125                                                               | 0.0125                                                                           | Fail (3% Rust).        |
| 0.0075                                                               | 0.015                                                                            | Fail (5% Rust).        |
| 0.025                                                                | 0.0125                                                                           | Pass (No Rust).        |

Table I shows that a surprisingly small amount of each of the ingredients can be used in combination to give effective rust inhibition. These small amounts in combination are equal or superior to substantially larger amounts of each of the components used separately.

## EXAMPLE II

In some lubricating oils it is desirable to use zinc dialkyl dithiophosphate as an antioxidant or extreme pressure additive. Some rust inhibitors of the free carboxylic acid type, including some very similar to the highly branched alkyl mercaptoacetic acid disclosed herein, form precipitates in the presence of zinc dialkyl dithiophosphate, giving hazy blends and a partial loss of rust protection. No such precipitate is formed by the use of the highly branched mercaptoacetic acid (C<sub>13</sub> Oxo SCH<sub>2</sub>COOH) shown in the table below. The table shows a comparison between branched C<sub>13</sub>H<sub>27</sub>SCH<sub>2</sub>COOH and a mercaptoacetic acid averaging n-C<sub>13</sub>H<sub>27</sub>SCH<sub>2</sub>COOH, where the alkyl groups range from n-C<sub>10</sub>H<sub>21</sub> to n-C<sub>18</sub>H<sub>37</sub>.

Table II  
HAZE TEST

| Blend                  | ZDDP | n-C <sub>13</sub> S <sup>1</sup> Acetic Acid | C <sub>13</sub> Oxo <sup>2</sup> S Acetic Acid | Appearance Approx. 60 Hrs. After Blending |
|------------------------|------|----------------------------------------------|------------------------------------------------|-------------------------------------------|
| Base Oil of Example I. |      |                                              |                                                | Bright.                                   |
| Do.                    | .05  | .01                                          |                                                | Do.                                       |
| Do.                    | .10  | .01                                          |                                                | Hazy.                                     |
| Do.                    | .20  | .005                                         |                                                | Do.                                       |
| Do.                    | .20  | .01                                          |                                                | Do.                                       |
| Do.                    | .05  | .02                                          |                                                | Do.                                       |
| Do.                    | .35  | .03                                          |                                                | Bright.                                   |
| Do.                    | .5   | .24                                          |                                                | Do.                                       |
| Do.                    | 3.0  | 3.0                                          |                                                | Do.                                       |

<sup>1</sup> Mixture of mercaptoacetic acids ranging from n-C<sub>10</sub>H<sub>21</sub>SCH<sub>2</sub>COOH to n-C<sub>18</sub>H<sub>37</sub>SCH<sub>2</sub>COOH and averaging n-C<sub>13</sub>H<sub>27</sub>SCH<sub>2</sub>COOH.

<sup>2</sup> This additive is the same C<sub>13</sub> Oxo mercaptoacetic acid as used in Example I.

## EXAMPLE III

The same base oil was used as in Example I. Samples were made up with 0.35 weight percent of a zinc dialkyl dithiophosphate (where the alkyl groups are derived from a mixture of about 25 weight percent isopropyl alcohol and about 75 weight percent methyl isobutylcarbinol) to test the effectiveness of the rust inhibiting combination.

The results are shown in Table III.

Table III

| Highly Branched (C <sub>13</sub> Oxo SCH <sub>2</sub> COOH) Mercaptoacetic Acid (Weight percent) <sup>1</sup> | Ba Salt of (C <sub>6</sub> ) <sub>2</sub> Naphthalene Sulfonate (Weight percent) <sup>2</sup> | MIL-L-17331A Rust Test |
|---------------------------------------------------------------------------------------------------------------|-----------------------------------------------------------------------------------------------|------------------------|
| 0.04                                                                                                          | Nil                                                                                           | Fail (2% Rust).        |
| 0.06                                                                                                          | Nil                                                                                           | Fail (1% Rust).        |
| Nil                                                                                                           | 0.05                                                                                          | Fail (10% Rust).       |
| Nil                                                                                                           | 0.10                                                                                          | Fail (<1% Rust).       |
| Nil                                                                                                           | 0.125                                                                                         | Pass (No Rust).        |
| .02                                                                                                           | 0.05                                                                                          | Pass (No Rust).        |

<sup>1</sup> This additive is the same mercaptoacetic acid as used in Example I.

<sup>2</sup> This additive is the same sulfonate as used in Example I.

## 4

Table II points out that the combination of mercaptoacetic acid and sulfonate in accordance with the present invention gives equally effective rust inhibition to oils containing zinc thiophosphate additives. The table also points out that the combination permits good rust inhibition at relatively low total rust inhibitor content and with a low level of free acid present. Thus, even when an excess of the inhibitors has been added as a margin of safety, the combination gives desirable flexibility in preparing blends to fulfill other important requirements of quality, for example, low ash and low neutralization number.

To demonstrate an interaction between rust-inhibiting components, low limiting concentrations, borderline in effectiveness, were tested experimentally. In actual service, however, it is desirable to use concentrations of rust inhibitors which will provide some margin of safety, concentrations which will still afford protection after some rust inhibitor has been removed as by plating out on metal surfaces or by very slow leaching of the inhibitors from the oil into water. The following examples show finished oil formulations incorporating the rust inhibitor combination of the invention in concentrations suitable for commercial service.

## EXAMPLE IV

A marine extreme pressure turbine oil was formulated using a paraffinic type oil derived from a Mid-Continent crude by distillation, phenol extraction, MEK dewaxing with methyl ethyl ketone and clay contacting.

This base oil had the same physical properties as shown in Example I.

The following ingredients were added to this base oil. 0.35 weight percent of the zinc dialkyl dithiophosphate cited in Example III; 0.05 weight percent of barium dinonylnaphthalene sulfonate (as 50% concentrate in Coastal oil) prepared as in Example I; 0.03 weight percent C<sub>13</sub> Oxo mercaptoacetic acid prepared as in Example I; 0.0005 weight percent Silicone antifoam agent (350 centistokes at 25° C.).

The finished inhibited formulation had the following inspections.

|                                                                  |                 |
|------------------------------------------------------------------|-----------------|
| Viscosity, S.U.S., at 210° F.                                    | 59.3.           |
| Viscosity, S.U.S., at 100° F.                                    | 397.7.          |
| Viscosity index                                                  | 104.5.          |
| Pour point, ° F.                                                 | 20.             |
| Neutralization number (ASTM D974)                                | 0.81.           |
| Sea water rust test (MIL-L-17331A)                               | Pass (no rust). |
| Oxidation life (ASTM D943)                                       | 1000 hrs.       |
| Emulsion test (ASTM D1401) (3 ml. max. lacy cuff after 25 mins.) | Pass.           |
| Mineral acidity (MIL-L-17331A)                                   | Neutral.        |
| Copper strip corrosion (ASTM D130) (3 hours at 212° F.)          | 1(a).           |
| Conradson carbon (ASTM D189)                                     | 0.16.           |
| Sulfated ash                                                     | 0.14.           |
| Tag Robinson color                                               | 13 1/4.         |
| Mean Hertz load (VV-L-791, 6503)                                 | 35.2 kg.        |
| Ryder gear test (MIL-L-17331A)                                   | 3310 lbs./inch. |
| Four ball wear scar (15 kg., 80° C., 600 r.p.m., 2 hrs.)         | 0.27 mm.        |

This turbine oil is being field tested in a new 38,000 ton supertanker equipped with a 26,500 rated shaft horsepower compounded steam turbine, built by Newport News Shipbuilding & Dry Dock Company. The steam turbine is coupled to an articulated double reduction main propulsion gear set built by General Electric Company. The turbine oil has shown excellent service in this test.

## EXAMPLE V

A higher viscosity lubricating oil was prepared by blending about 80 weight percent of the base oil of Example I with about 20 weight percent of a (propane) de-

asphalted, MEK dewaxed, phenol extracted, clay contacted residuum from a Mid-Continent crude to give a base oil having a viscosity at 210° F. of about 65 S.U.S. To this base oil was added 0.34 weight percent zinc dialkyl dithiophosphate, 0.15 weight percent barium dinonylnaphthalene sulfonate, and 0.05 weight percent  $C_{13}$  Oxo mercaptoacetic acid. This oil passed the ASTM D665 sea water rust test.

Similar oils of higher viscosity containing: (a) 0.05 sulfonate and 0.03  $C_{13}$  Oxo  $SC_2COOH$  or; (b) 0.10 sulfonate and 0.04  $C_{13}$  Oxo  $SC_2COOH$  have passed the above rust test.

The following claims set forth that part of the above described invention for which patent protection is respectfully requested.

What is claimed is:

1. A non-emulsifying lubricating composition comprising a major proportion of a mineral lubricating oil and in the range of 0.005 to 1.0 weight percent each of a branched  $C_9$  to  $C_{17}$  alkyl mercaptoacetic acid and an alkaline earth metal salt of  $C_6$  to  $C_{12}$  branched chain dialkyl-naphthalene sulfonate as the sole sulfonate, the alkaline earth metal being selected from the group consisting of calcium and barium.

2. The lubricating composition of claim 1 comprising, in addition thereto, 0.05 to 2.0 weight percent of an oil-soluble zinc  $C_2$  to  $C_{18}$  dialkyl dithiophosphate.

3. The lubricating composition according to claim 1 wherein the alkyl radical of the alkyl mercaptoacetic

acid is a highly branched radical having at least three branched groups.

4. The lubricating composition according to claim 1 wherein the mercaptoacetic acid is a highly branched  $C_{13}$  mercaptoacetic acid and the sulfonate is a branched chain dinonylnaphthalene sulfonate.

5. The lubricating composition according to claim 1 wherein said alkyl mercaptoacetic acid is a  $C_{13}$  Oxo mercaptoacetic acid and wherein said dialkyl naphthalene sulfonate is a barium dinonylnaphthalene sulfonate.

6. The lubricating composition according to claim 2 wherein said alkyl mercaptoacetic acid is a  $C_{13}$  Oxo mercaptoacetic acid and wherein said dialkyl naphthalene sulfonate is a barium dinonylnaphthalene sulfonate.

15

References Cited in the file of this patent

UNITED STATES PATENTS

|           |               |                |
|-----------|---------------|----------------|
| 2,364,284 | Freuler       | Dec. 5, 1944   |
| 2,491,066 | Wasson et al. | Dec. 13, 1949  |
| 2,693,448 | Landis et al. | Nov. 2, 1954   |
| 2,739,125 | Myers et al.  | Mar. 20, 1956  |
| 2,764,548 | King et al.   | Sept. 25, 1956 |
| 2,779,784 | Sharrah       | Jan. 29, 1957  |

25

FOREIGN PATENTS

|         |               |               |
|---------|---------------|---------------|
| 659,072 | Great Britain | Oct. 17, 1951 |
| 689,759 | Great Britain | Apr. 1, 1953  |
| 526,206 | Canada        | June 12, 1956 |